

## UNITED STATES PATENT OFFICE

ALBERT C. FISCHER, OF CHICAGO, ILLINOIS, ASSIGNOR TO THE PHILIP CAREY MANUFACTURING COMPANY, A CORPORATION OF OHIO

## CONSTRUCTIONAL MATERIAL

No Drawing.

Application filed August 15, 1927. Serial No. 213,182.

This invention relates to constructional material, such as, roofing material, insulating material, tapes, shingles, packing and the like.

5 The object of my present invention is to provide such constructional materials with an adhesive coating which is normally sticky or tacky to the touch and which lastingly maintains this mastic condition whereby the 10 material may be packed and stored for long periods of time without losing its tackiness and may be transported to its place of installation and used in such tacky condition without further treatment.

15 A further object of my invention resides in the application of this normally lastingly adhesive, sticky to the touch, to sheets or strips of carrier material, hereinafter called vehicles, so that when rolled into package form or placed face to face in contact with a similar sheet for packing and storing and transportation, they may be unrolled or pulled apart readily without tearing or damaging, and can be installed in tacky condition; in 20 this instance the tacky coating permits the facile separation of the contacting vehicle surfaces, the line of cleavage passing through the mastic itself. The vehicle thus provided 25 with a lasting adhesive, mastic coating is particularly adapted to act as a packing for various types of installations, not only because of the waterproofing quality of the mastic but also because of its pronounced and lasting quality of adhesiveness and further because of its plasticity.

30 A further object of the present invention resides in the utilization of means for maintaining or insuring the lasting quality of the adhesive by saturating the vehicle with an oil and particularly a non-drying oil which not only prevents the oil contained in the adhesive coating from penetrating too far into the vehicle and being absorbed, which 35 detracts from the tackiness of the coating, but also which serves slowly to unite, or in the use of other oils not to unite, with the oil with which the substance of the coating is fluxed, whereby to maintain the coating in 40 its normal, tacky, mastic condition, sticky

to the touch and soft and pliable for long periods of time; practically indefinitely.

In the present invention the vehicle may consist of sheets, strips, or slabs of tar paper, 55 felt, fabric, fibers or other preferred material.

The saturant for the vehicle consists of an oil or combination of oils. I preferably, in the present application, saturate the vehicle with a non-drying oil, such as, cotton seed 60 oil, rape seed oil, castor oil or other similar oil in treated or untreated form.

The oil acts as a waterproofing filler for the vehicle. The vehicle saturated with this non-drying oil may then have applied thereto an adhesive, which may be of any preferred kind. The fact that the vehicle is saturated with the oil will prevent the deep penetration 65 of the adhesive into the body of the vehicle and at the same time the oil will prevent the drying out of the adhesive, whereby 70 said adhesive will continue for long periods of time in its mastic state, tacky to the touch.

The saturant of the vehicle forms a slow 75 union of junction with the coating of bituminous matter which contains or is fluxed with an oil or oils that will unite with the saturant of the vehicle.

Alternatively, in some instances the coating of bituminous material is fluxed with 80 mineral oil, which will not unite with the saturant of the vehicle.

The tendency of the saturant is to keep the bituminous material of the coating in a thoroughly mastic state where the substances 85 will unite, and in a pliable, soft state where they do not unite.

Castor oil may be used as a saturant for the vehicle where the coating materials contain mineral oils and where no union of the 90 oil of the saturant and the oil of the coating is desired. The coating material may be a high melting point bituminous substance with mineral oils, or the coating may be any combination of flux oils, mineral, vegetable 95 or animal oils.

The coating with which the vehicle is thus saturated on either one or both sides preferably comprises a slow drying, tacky bituminous, vegetable or animal substance or com- 100

bination of two or more; which approximates the following specifications, or may be more or less fluid.

1. The consistency at 77 degrees F. should be below 7.0.

5. 2. The susceptibility factor should be as low as possible, preferably under 25.

3. The ductility at 77 degrees F. should be as high as possible and preferably over 25 centimeters.

10 4. Fusing point by K & S method should be between 80 degrees and 100 degrees F.

5. It should appear tacky and adhesive at normal temperature and retain this property as long as possible on exposure to air.

15 This formula is merely a standard and other formulas more or less fluid may be used with or without a suitable filler as a flow retarder, or the flow tendency may be stopped by using a non-flowing gummy substance in combination.

It will be understood that my invention contemplates constructional material, the adhesiveness of which serves to hold said material in place in distinction to other materials which involve the use of pitch, or other material, mopped on at the time of assembling the material. This is especially true in the application of the invention to roofing sheets, 30 for the purpose of holding the sheets of roofing material in place. It will be understood that after two sheets of building material according to the present invention have been separated, the adhesive surface of one sheet 35 will be placed in contact with the non-adhesive surface of another sheet. The adhesive or mastic will cause a union with non-adhesive surfaces to which it is applied, which union may be made very excellent by means of 40 rolling and which will improve in the course of time.

It will also be understood that if it should be found that the adhesive surface of a sheet should become dried out, a solvent such as 45 toluol, benzol, kerosene, or cotton oil, may be used to bring the sheet back into adhesive state.

The subject matter of this case has been withdrawn from my Patent, No. 1,550,310, 50 issued August 18, 1925.

I claim:

1. A vehicle saturated with an oil and coated with a mastic of lasting adhesiveness, sticky to the touch.

55 2. A vehicle saturated with a non-drying oil and coated with a mastic of lasting adhesiveness and sticky to the touch.

3. Constructional material comprising a vehicle saturated with an oil and coated with 60 a waterproofing mastic of lasting adhesiveness fluxed with an oil which forms a slow union with the vehicle saturant.

4. Constructional material comprising a vehicle saturated with an oil and coated with 65 a bituminous mastic, the oil saturant serv-

ing to maintain the mastic in a soft, lastingly adhesive condition.

5. Constructional material comprising a sheet of roofing felt saturated with oil and coated with bituminous adhesive maintained 70 in a condition of lasting stickiness by the oil saturant.

6. Constructional material comprising a vehicle saturated with an oil, and coated with a bituminous material fluxed with a mineral 75 oil which does not unite with the oil saturant whereby to keep the mastic in a soft, pliable, lasting state of adhesiveness.

Signed at Chicago, Illinois, this 9th day of August 1927.

ALBERT C. FISCHER.